

3,729,417

## QUENCHING OIL COMPOSITIONS

Kametaro Hashimoto and Hiroo Nakamura, Toyota-shi, Toshio Okada, Kyoto-fu, and Misugu Tanaka and Kazuto Fukuhara, Kobe-shi, Japan, assignors to Toyota Jidosha Kogyo Kabushiki Kaisha, Toyota-shi, Aichi-ken, and Nippon Grease Co., Ltd., Dojima, Kitaku, Osaka-shi, Japan

No Drawing. Filed Feb. 12, 1970, Ser. No. 10,990  
Claims priority, application Japan, Feb. 14, 1969,  
44/11,199

Int. Cl. C10m 1/48

U.S. CL. 252—46.6

3 Claims

### ABSTRACT OF THE DISCLOSURE

Quenching oil composition of the invention comprises mineral quenching oil containing a specific compound belonging to (1) aliphatic acids or derivatives thereof, (2) phosphites, (3) thiophosphites, (4) phosphates, (5) zinc dialkyl dithiophosphates, (6) disulfides, (7) tetraalkylthiuram sulfides, (8) dithiocarbamates or (9) mercaptanes, said compound being contained in the range of 0.05 to 5 weight parts, based on 100 weight parts of the mineral quenching oil. The present quenching oil compositions are capable of quenching metals and, at the same time, imparting lubricating property to the metals quenched therewith.

This invention relates to new and useful quenching oil compositions and to the method of quenching metals therewith.

Hardening metals such as steel by quenching operation is well known in the art and various quenching oil compositions have been proposed for the purpose. By employing known compositions, however, the hardness of the metal quenched therewith increases but no lubricating property is imparted to the metal surface. In the prior method, therefore, the metal products hardened by quenching operation are further subjected to lubricating treatment whenever such property is required. Bolts used for securing a member to which high valuable stress is applied, for example, must effect a high order of fastening force, and therefore, after being hardened by quenching operation and washed with trichloroethylene, they are subsequently subjected to surface treatment to render the surface thereof lubricious. Thus the prior methods require two separate procedures and apparatuses for hardening the metal and for imparting lubricity to the metal. As far as the applicants are aware, no attempts have been heretofore made to obtain quenching oil compositions capable of quenching and at the same time imparting lubricating property to the metal surface quenched therewith.

One object of the invention is to provide a quenching oil composition whereby not only the hardness of metal quenched therewith is increased but also excellent lubricity can be imparted to the surface thereof.

Another object of the invention is to provide a quenching oil composition which makes it possible to conduct the step of hardening metal and, at the same time, the step of surface treatment of the metal for lubricity.

These and other objects and advantages of the invention will be apparent from the following description.

According to the researches of the present inventors it has now been found that when a specific compound is added to a conventional quenching oil of mineral origin in a predetermined amount and metal to be hardened is quenched with the resultant composition the hardness of the metal thus treated is increased and excellent lubricity is simultaneously imparted to the metal surface.

The specific compounds which display the above effect and which are used in the invention are classified into nine groups to follow:

(1) An aliphatic acid compound having the formula of



wherein  $R^1$  is hydrogen, an alkyl of 15 to 17 carbon atoms or  $C_{17}H_{35}-$ ,  $R^2$  is hydrogen, a lower alkyl of 1 to 6 carbon atoms, Cu (II) or Cd (II), and  $m$  is an integer of 1 when  $R^2$  is hydrogen or a lower alkyl or an integer of 2 when  $R^2$  is Cu or Cd;

(2) A phosphite having the formula of



wherein  $R^3$  is hydrogen, an alkyl of 4 to 12 carbon atoms,  $C_{18}H_{35}-$ , phenyl or an alkyl ( $C_1-C_9$ ) phenyl but all of the  $R^3$  are not hydrogen;

(3) A thiophosphite having the formula of



wherein  $R^4$  is an alkyl of 10 to 13 carbon atoms,  $R^5$  is phenyl or methyl phenyl,  $n$  is an integer of 1 to 3 and  $p$  is 0 when  $n$  is 3, an integer of 1 when  $n$  is 2 or an integer of 2 when  $n$  is 1;

(4) A phosphate having the formula of



wherein  $R^6$  is an alkyl of 1 to 9 carbon atoms,  $\beta$ -chloroalkyl of 1 to 4 carbon atoms,  $C_{18}H_{35}-$ , phenyl or methyl phenyl,  $q$  is an integer of 1 to 3,  $r$  is 0 when  $q$  is 3, an integer of 1 when  $q$  is 2 or an integer of 2 when  $q$  is 1;

(5) A zinc dialkyl dithiophosphate having the formula of



wherein  $R^7$  is an alkyl of 1 to 12 carbon atoms;

(6) A disulfide having the formula of



wherein  $R^8$  is an alkyl of 1 to 12 carbon atoms, phenyl or benzyl;

(7) A tetraalkylthiuram sulfide



wherein  $R^9$  is a lower alkyl of 1 to 4 carbon atoms and  $v$  is an integer of 1 to 2;

(8) A dithiocarbamate having the formula of



wherein  $R^{10}$  is an alkyl of 1 to 12 carbon atoms, phenyl or an alkyl ( $C_1-C_4$ ) phenyl,  $M$  is a divalent or trivalent metal, and  $w$  is an integer of 2 when  $M$  is divalent metal or an integer of 3 when  $M$  is trivalent metal; and

(9) A mercaptane having the formula of



wherein  $R^{11}$  is an alkyl of 8 to 18 carbon atoms or phenyl.

Though any compounds belonging to the above groups (I) to (IX) can be effectively used in the invention,

phosphites, thiophosphites, phosphates, zinc dialkyl dithiophosphates and dithiocarbamates are particularly desirable. Representative examples of aliphatic acid compounds of the Formula I are formic acid, ethyl formate, isoamyl formate, palmitic acid, heptadecanoic acid, stearic acid, cadmium stearate, oleic acid, ethyl oleate and cupric oleate. Of these formic acid, isoamyl formate, palmitic acid, heptadecanoic acid, cadmium stearate, oleic acid, ethyl oleate and cupric oleate are preferable, the most desirable being heptadecanoic acid. Examples of phosphites of the Formula II are dibutyl hydrogenphosphite, tributyl phosphite, trioctyl phosphite, bis(2-ethylhexyl) hydrogenphosphite, tri(2-ethylhexyl) phosphite, tridecyl phosphite, dilauryl hydrogenphosphite, tri-lauryl phosphite, trioleil phosphite, triphenyl phosphite, tricresyl phosphite, tris(nonylphenyl) phosphite, diphenyl nonylphenyl phosphite and phenyl diisodecyl phosphite. Of these tributyl phosphite, trioctyl phosphite, tridecyl phosphite, dilauryl hydrogenphosphite, trioleil phosphite, triphenyl phosphite, tricresyl phosphite, diphenyl-nonylphenyl phosphite, tris(nonylphenyl) phosphite and phenyl diisodecyl phosphite are preferable, the most desirable being dilauryl hydrogenphosphite, triphenyl phosphite, tricresyl phosphite and tris(nonylphenyl) phosphite. Examples of thiophosphites of the Formula III are tridecyl trithiophosphite, phenyl dilauryl dithiophosphite, diphenyl lauryl monothiophosphite and tri-lauryl trithiophosphite. Of these phenyl dilauryl dithiophosphite, diphenyl lauryl monothiophosphite and tri-lauryl trithiophosphite are preferable, the most desirable being phenyldilauryl dithiophosphite and diphenyl lauryl monothiophosphite. Examples of phosphates of the Formula IV are monomethyl phosphate, dimethyl phosphate, diethyl phosphate, diisopropyl phosphate, monobutyl phosphate, dibutyl phosphate, mono-octyl phosphate, dioctyl phosphate,  $\beta$ -chloroethyl phosphate, di( $\beta$ -chloroethyl) phosphate, dioleil phosphate, trioleil phosphate, triphenyl phosphate, tricresyl phosphate and bis(2-ethylhexyl) phosphate. Of these monomethyl phosphate, dimethyl phosphate, mono-butyl phosphate, dibutyl phosphate, mono-octyl phosphate, dioctyl phosphate, mono( $\beta$ -chloroethyl) phosphate, di( $\beta$ -chloroethyl) phosphate, trioleil phosphate, triphenyl phosphate, tricresyl phosphate and bis(2-ethylhexyl) phosphate are preferable, the most desirable being a 9:1-1:9 weight ratio mixture of monomethyl phosphate and dimethyl phosphate as well as a 9:1-1:9 weight ratio mixture of mono-octyl phosphate and dioctyl phosphate. Examples of zinc dialkyl dithiophosphates of the Formula V are zinc dipropyl dithiophosphate, zinc dibutyl dithiophosphate, zinc dipentyl dithiophosphate, zinc dihexyl dithiophosphate, zinc di-octyl dithiophosphate, zinc didecyl dithiophosphate and zinc dilauryl dithiophosphate. Of these zinc dipropyl dithiophosphate, zinc dibutyl dithiophosphate, zinc dipentyl thiophosphate, zinc dihexyl dithiophosphate, zinc dioctyl dithiophosphate, zinc didecyl dithiophosphate, and zinc dilauryl dithiophosphate are preferable, the most desirable being zinc dihexyl dithiophosphate. Examples of disulfides of the Formula VI are di-n-propyl disulfide, di-n-butyl disulfide, diteriarybutyl disulfide, di-n-pentyl disulfide, diteriaryhexyl disulfide, diteriaryoctyl disulfide, dilauryl disulfide, diphenyl disulfide and dibenzyl disulfide. Of these diteriarybutyl disulfide, dilauryl disulfide, diphenyl disulfide and dibenzyl disulfide are preferable, the most desirable being diteriarybutyl disulfide. Examples of tetraalkyl thiuram sulfides of the Formula VII are tetramethyl thiuram disulfide, tetramethyl thiuram monosulfide, tetraethyl thiuram disulfide, tetrapropyl thiuram disulfide, tetrabutyl thiuram disulfide. Of these tetramethyl thiuram disulfide, tetraethyl thiuram disulfide and tetramethyl thiuram monosulfide are preferable, the most desirable being tetramethyl thiuram disulfide. Examples of dithiocarbamates of the Formula VIII are ferric dimethyl dithiocarbamate, cupric dimethyl dithiocarbamate, zinc dimethyl dithiocarbamate, zinc diethyl dithiocarbamate, zinc dipropyl dithiocarbamate, zinc dibutyl dithiocarbamate, zinc dihexyl dithiocarbamate, zinc di-octyl dithiocarbamate, zinc didecyl dithiocarbamate, zinc dilauryl dithiocarbamate, cadmium dimethyl dithiocarbamate, cadmium dipentyl dithiocarbamate, cadmium dihexyl dithiocarbamate, cadmium di-octyl dithiocarbamate, cadmium didecyl dithiocarbamate, cadmium dilauryl dithiocarbamate, lead dipropyl dithiocarbamate, lead dibutyl dithiocarbamate, lead dipentyl dithiocarbamate, lead dihexyl dithiocarbamate, lead dioctyl dithiocarbamate, lead didecyl dithiocarbamate, lead dilauryl dithiocarbamate, lead diphenyl dithiocarbamate, antimony dipropyl dithiocarbamate, antimony dibutyl dithiocarbamate, antimony dipentyl dithiocarbamate, antimony dihexyl dithiocarbamate, antimony di-octyl dithiocarbamate, antimony didecyl dithiocarbamate, antimony dilauryl dithiocarbamate and zinc ethylphenyl dithiocarbamate. Of these ferric dimethyl dithiocarbamate, cupric dimethyl dithiocarbamate, zinc dimethyl dithiocarbamate, zinc diethyl dithiocarbamate, zinc dipentyl dithiocarbamate, cadmium dipentyl dithiocarbamate, lead dipentyl dithiocarbamate, antimony dipentyl dithiocarbamate and zinc ethylphenyl dithiocarbamate are desirable, the most preferable being cadmium dipentyl dithiocarbamate. Preferable examples of mercaptanes of the Formula IX are n-octyl mercaptane, n-dodecyl mercaptane, cetyl mercaptane, stearyl mercaptane, thiophenol and benzyl mercaptane. Of these benzyl mercaptane is most preferable.

30 The above compounds are added, alone or in mixture of more than 2 species to mineral quenching oil in the amount of 0.05 to 5 weight parts, based on 100 weight parts of the quenching oil. The resultant composition of the invention is not only effective as quenching oil but also imparts lubricating property to the surface of the metal quench therewith. The theoretical reason why the lubricating property is imparted to the metal surface treated with the present composition has not been made clear yet, but it is supposed that by the addition of the specific compound as above the metal treated with the present composition is covered with lubricating film which renders the metal surface lubricious. When the amount of the compound added is less than 0.05 weight part per 100 weight parts of quenching oil the resultant composition displays poor effect in rendering the metal surface treated therewith lubricious, while the composition containing more than 5 weight parts of the compound per 100 weight parts of quenching oil displays no better effect but rather adversely affects the cooling property and stability of the oil. Though preferable amount of the compound varies in accordance with the kinds of the compounds used, usually it is in the range of 0.1 to 2 weight parts, based on 100 weight parts of the quenching oil.

35 The quenching oils used in the invention are mineral oils obtained as distillates from various types of crude oils such as paraffinic or naphthenic crudes. The oils may have a flash point of higher than 160° C., preferably in the range of 170 to 300° C., and a viscosity of more than 45 RW sec. at 50° C., preferably in the range of 50 to 150 RW sec. at 50° C.

40 Hardening metals such as steel may be made by any methods of quenching operation known in the art. In general it is conducted by heating the metal to a temperature higher than its critical temperature and quenching the metal by immersion in the present quenching oil composition. The present composition may also be used for quenching of tempered metal, whereby more excellent lubricity may be imparted to the metal surface. In using the present composition it is preferable to heat metal in an atmosphere containing no oxygen, such as in nitrogen or carbon dioxide gas atmosphere, since the presence of oxygen reduces the lubricity of the resultant metal.

For better understanding of the invention examples are given below.

## EXAMPLE 1

Seventeen kinds of quenching oil compositions were prepared by adding fatty acid compounds shown in Table 1 below in predetermined amount to 100 weight parts of mineral quenching oil having a viscosity of 59.8 RW sec. at 50° C. and a flash point of 178° C.

Roller pins of 2.0 mm. in diameter and 29.9 mm. in length were heated at 850° C. for 10 minutes in an atmosphere of 9:1 volume ratio mixture of argon and hydrogen. The respective pins thus treated were immediately immersed in respective quenching oil compositions at 80° C. for 5 minutes, then washed with trichloroethylene and dried.

The lubricity of the roller pins thus obtained was tested by the method described in "Jukuuke Junkatsu Binran," pp. 773-775 (1961) published by Nikkan Kogyo Shinbunsha, Japan. In this method the roller pin to be tested was rotatably supported by means of steel balls and the based portion of a pendulum was fixed to the pin so as to allow the pendulum to swing integrally with the pin. To test the lubricity of the pin, the pendulum was swung in an atmosphere heated to 50° C. and the amplitude of the first stroke of swing and that of the fifth stroke were respectively measured. The coefficient of boundary friction was given by the following equation:

$$f = 3.2 \times \frac{A_0 - A_5}{5}$$

wherein  $f$  is coefficient of boundary friction,  $A_0$  is amplitude of the first stroke and  $A_5$  is amplitude of the fifth stroke.

The results of the measurement are shown in Table 1 below.

TABLE 1

| Comp. No. | Fatty acid compounds added |                                                                  | Amount added<br>(wt. parts) | Coefficient of boundary<br>(at 50° C.) |
|-----------|----------------------------|------------------------------------------------------------------|-----------------------------|----------------------------------------|
|           | Name                       | Formula                                                          |                             |                                        |
| 1-A-1     | Formic acid                | HCOOH                                                            | 1.0                         | 0.3341                                 |
| 1-A-2     | do                         | HCOOH                                                            | 2.0                         | 0.3277                                 |
| 1-A-3     | do                         | HCOOH                                                            | 3.0                         | 0.2906                                 |
| 1-B-1     | Isoamyl formate.           | HCOOC <sub>5</sub> H <sub>11</sub>                               | 1.0                         | 0.2637                                 |
| 1-B-2     | do                         | HCOOC <sub>5</sub> H <sub>11</sub>                               | 2.0                         | 0.2918                                 |
| 1-B-3     | do                         | HCOOC <sub>5</sub> H <sub>11</sub>                               | 3.0                         | 0.3443                                 |
| 1-C-1     | Palmitic acid.             | C <sub>15</sub> H <sub>31</sub> COOH                             | 1.0                         | 0.3392                                 |
| 1-C-2     | do                         | C <sub>15</sub> H <sub>31</sub> COOH                             | 2.0                         | 0.3392                                 |
| 1-C-3     | do                         | C <sub>15</sub> H <sub>31</sub> COOH                             | 3.0                         | 0.3341                                 |
| 1-D-1     | Heptadecanoic acid.        | C <sub>17</sub> H <sub>33</sub> COOH                             | 1.0                         | 0.2686                                 |
| 1-D-2     | do                         | C <sub>17</sub> H <sub>33</sub> COOH                             | 2.0                         | 0.2573                                 |
| 1-E-1     | Cadmium stearate.          | (C <sub>17</sub> H <sub>33</sub> COO) <sub>2</sub> Cd            | 1.0                         | 0.41112                                |
| 1-F-1     | Oleic acid                 | C <sub>17</sub> H <sub>33</sub> COOH                             | 0.5                         | 0.41856                                |
| 1-F-2     | do                         | C <sub>17</sub> H <sub>33</sub> COOH                             | 1.0                         | 0.40326                                |
| 1-G-1     | Ethyl oleate.              | C <sub>17</sub> H <sub>33</sub> COOC <sub>2</sub> H <sub>5</sub> | 1.0                         | 0.41946                                |
| 1-H-1     | Cupric oleate.             | (C <sub>17</sub> H <sub>33</sub> COO) <sub>2</sub> Cu            | 0.5                         | 0.34048                                |
| 1-H-2     | do                         | (C <sub>17</sub> H <sub>33</sub> COO) <sub>2</sub> Cu            | 1.0                         | 0.32384                                |
| Control   |                            |                                                                  | 0                           | 0.44032                                |

## EXAMPLE 2

Twenty-four kinds of quenching oil compositions were prepared by adding phosphites shown in Table 1 above in predetermined amount to 100 weight parts of mineral quenching oil the same as in Example 1.

Roller pins quenched with above compositions in the same manner as in Example 1 were measured to determine coefficient of boundary friction as in Example 1 with the results shown in Table 2 below.

TABLE 2

| Comp. No. | Phosphites added               |                                                                                                   | Amount added<br>(wt. parts) | Coefficient of boundary<br>friction<br>(at 50° C.) |
|-----------|--------------------------------|---------------------------------------------------------------------------------------------------|-----------------------------|----------------------------------------------------|
|           | Name                           | Formula                                                                                           |                             |                                                    |
| 2-A-1     | Tributyl phosphite             | (C <sub>4</sub> H <sub>9</sub> O) <sub>3</sub> P                                                  | 0.5                         | 0.41216                                            |
| 2-A-2     | do                             | (C <sub>4</sub> H <sub>9</sub> O) <sub>3</sub> P                                                  | 1.0                         | 0.23296                                            |
| 2-A-3     | do                             | (C <sub>4</sub> H <sub>9</sub> O) <sub>3</sub> P                                                  | 2.0                         | 0.33280                                            |
| 2-A-4     | do                             | (C <sub>4</sub> H <sub>9</sub> O) <sub>3</sub> P                                                  | 3.0                         | 0.33920                                            |
| 2-B-1     | Trioctyl phosphite             | (C <sub>8</sub> H <sub>17</sub> O) <sub>3</sub> P                                                 | 1.0                         | 0.39680                                            |
| 2-B-2     | do                             | (C <sub>8</sub> H <sub>17</sub> O) <sub>3</sub> P                                                 | 2.0                         | 0.39936                                            |
| 2-B-3     | do                             | (C <sub>8</sub> H <sub>17</sub> O) <sub>3</sub> P                                                 | 3.0                         | 0.28416                                            |
| 2-C-1     | Tridecyl phosphite             | (C <sub>13</sub> H <sub>27</sub> O) <sub>3</sub> P                                                | 2.0                         | 0.40064                                            |
| 2-D-1     | Dilauryl hydrogen phosphite    | (C <sub>12</sub> H <sub>25</sub> O) <sub>2</sub> POH                                              | 0.1                         | 0.40060                                            |
| 2-D-2     | do                             | (C <sub>12</sub> H <sub>25</sub> O) <sub>2</sub> POH                                              | 0.5                         | 0.23936                                            |
| 2-D-3     | do                             | (C <sub>12</sub> H <sub>25</sub> O) <sub>2</sub> POH                                              | 1.0                         | 0.07936                                            |
| 2-D-4     | do                             | (C <sub>12</sub> H <sub>25</sub> O) <sub>2</sub> POH                                              | 2.0                         | 0.13952                                            |
| 2-D-5     | do                             | (C <sub>12</sub> H <sub>25</sub> O) <sub>2</sub> POH                                              | 3.0                         | 0.23936                                            |
| 2-E-1     | Trioleil phosphite             | (C <sub>18</sub> H <sub>35</sub> O) <sub>3</sub> P                                                | 3.0                         | 0.36224                                            |
| 2-F-1     | Triphenyl phosphite            | (C <sub>6</sub> H <sub>5</sub> O) <sub>3</sub> P                                                  | 0.5                         | 0.29952                                            |
| 2-F-2     | do                             | Same as above                                                                                     | 1.0                         | 0.22144                                            |
| 2-F-3     | do                             | do                                                                                                | 2.0                         | 0.19968                                            |
| 2-F-4     | do                             | do                                                                                                | 3.0                         | 0.28288                                            |
| 2-G-1     | Tricresyl phosphite            | (C <sub>6</sub> H <sub>5</sub> O) <sub>3</sub> P                                                  | 0.5                         | 0.18944                                            |
| 2-G-2     | do                             | Same as above                                                                                     | 1.0                         | 0.17152                                            |
| 2-G-3     | do                             | do                                                                                                | 2.0                         | 0.17153                                            |
| 2-G-4     | do                             | do                                                                                                | 3.0                         | 0.17152                                            |
| 2-H-1     | Diphenyl nonylphenyl phosphite | (C <sub>6</sub> H <sub>5</sub> O) <sub>2</sub> PO-C <sub>2</sub> H <sub>11</sub>                  | 1.0                         | 0.23680                                            |
| 2-H-2     | do                             | Same as above                                                                                     | 2.0                         | 0.28680                                            |
| 2-H-3     | do                             | do                                                                                                | 3.0                         | 0.36608                                            |
| 2-I-1     | Tris(nonylphenyl phosphite)    | (C <sub>9</sub> H <sub>17</sub> -C <sub>6</sub> H <sub>5</sub> O) <sub>3</sub> P                  | 1.0                         | 0.18560                                            |
| 2-J-1     | Phenyl diisodecyl phosphite    | (C <sub>6</sub> H <sub>5</sub> -O-P(O <sub>2</sub> C <sub>10</sub> H <sub>21</sub> ) <sub>2</sub> | 3.0                         | 0.32128                                            |
| Control   |                                |                                                                                                   | 0                           | 0.44032                                            |

7  
EXAMPLE 3

Ten kinds of quenching oil compositions were prepared by adding thiophosphites shown in Table 3 below in predetermined amount to 100 weight parts of mineral quenching oil the same as in Example 1.

the same manner as in Example 1 were measured to determine coefficient of boundary friction as in Example 1 with the results shown in Table 4 below. In Table 4 the mixtures described in Compositions Nos. 4-A to 4-D mean 1:1 weight ratio mixtures of respective compounds.

5

8

TABLE 4

| Comp. No. | Name                                                                         | Phosphate added                                                                      | Amount added (wt. parts) | Coefficient of boundary friction (at 50° C.) |
|-----------|------------------------------------------------------------------------------|--------------------------------------------------------------------------------------|--------------------------|----------------------------------------------|
| 4-A-1     | Mixture—<br>(Dimethyl phosphate)<br>(Monomethyl phosphate)                   | $(CH_3O)_2P(O)OH$<br>$CH_3OP(O)(OH)_2$                                               | 0.1                      | 0.36608                                      |
| 4-B-1     | Mixture—<br>(Dibutyl phosphate)<br>(Monobutyl phosphate)                     | $(C_4H_9O)_2P(O)OH$<br>$C_4H_9OP(O)(OH)_2$                                           | 0.1                      | 0.17280                                      |
| 4-B-2     | Same as Comp. No. 4-B-1                                                      | Same as Comp. No. 4-B-1                                                              | 0.5                      | 0.13312                                      |
| 4-B-3     | do                                                                           | do                                                                                   | 1.0                      | 0.12544                                      |
| 4-C-1     | Mixture—<br>(Diethyl phosphate)<br>(Monooctyl phosphate)                     | $(C_8H_{17}O)_2P(O)OH$<br>$C_8H_{17}OP(O)(OH)_2$                                     | 0.1                      | 0.16640                                      |
| 4-C-2     | Same as Comp. No. 4-C-1                                                      | Same as Comp. No. 4-C-1                                                              | 0.5                      | 0.18432                                      |
| 4-C-3     | do                                                                           | do                                                                                   | 1.0                      | 0.22016                                      |
| 4-C-4     | do                                                                           | do                                                                                   | 2.0                      | 0.23552                                      |
| 4-C-5     | do                                                                           | do                                                                                   | 3.0                      | 0.30080                                      |
| 4-D-1     | Mixture—<br>(Di(β-chloroethyl) phosphate)<br>(Mono(β-chloroethyl) phosphate) | $(ClCH_2CH_2O)_2P(O)OH$<br>$ClCH_2CH_2OP(O)(OH)_2$                                   | 0.1                      | 0.23808                                      |
| 4-D-2     | Same as Comp. No. 4-D-1                                                      | Same as Comp. No. 4-D-1                                                              | 0.5                      | 0.20224                                      |
| 4-D-3     | do                                                                           | do                                                                                   | 1.0                      | 0.29922                                      |
| 4-E-1     | Trioleil phosphate                                                           | $(C_{18}H_{35}O)_3PO$                                                                | 1.0                      | 0.21888                                      |
| 4-E-2     | do                                                                           | $(C_{18}H_{35}O)_2PO$                                                                | 2.0                      | 0.23424                                      |
| 4-E-3     | do                                                                           | $(C_{18}H_{35}O)_3P(O)$                                                              | 3.0                      | 0.24704                                      |
| 4-F-1     | Triphenyl phosphate                                                          |    | 1.0                      | 0.3379                                       |
| 4-F-2     | do                                                                           | Same as above                                                                        | 2.0                      | 0.3764                                       |
| 4-F-3     | do                                                                           | do                                                                                   | 3.0                      | 0.3789                                       |
| 4-G-1     | Tricresyl phosphate                                                          |  | 1.0                      | 0.3123                                       |
| 4-G-2     | do                                                                           | Same as above                                                                        | 2.0                      | 0.2726                                       |
| 4-G-3     | do                                                                           | do                                                                                   | 3.0                      | 0.3072                                       |
| 4-H-1     | Bis(2-ethylhexyl) phosphate                                                  | $(C_8H_{17}O)_2P(O)OH$                                                               | 0.5                      | 0.2726                                       |
| 4-H-2     | do                                                                           | $(C_8H_{17}O)_2P(O)OH$                                                               | 1.0                      | 0.2445                                       |
| 4-H-3     | do                                                                           | $(C_8H_{17}O)_3P(O)OH$                                                               | 2.0                      | 0.2253                                       |
| Control   |                                                                              |                                                                                      | 0                        | 0.44032                                      |

Roller pins quenched with above compositions in the same manner as in Example 1 were measured to determine coefficient of boundary friction as in Example 1 with the results shown in Table 3 below.

45

Thirty-two kinds of quenching oil compositions were prepared by adding zinc dialkyl dithiophosphates shown in Table 5 below in predetermined amount to 100 weight parts of mineral quenching oil the same as in Example 1.

TABLE 3

| Comp. No. | Name                             | Thiophosphate added                              | Amount added (wt. parts) | Coefficient of boundary friction (at 50° C.) |
|-----------|----------------------------------|--------------------------------------------------|--------------------------|----------------------------------------------|
| 3-A-1     | Phenyl dilauryl dithiophosphate  | $(C_{12}H_{25}S)_2P-O-\text{C}_6H_5$             | 0.5                      | 0.20224                                      |
| 3-A-2     | do                               | Same as above                                    | 1.0                      | 0.17408                                      |
| 3-A-3     | do                               | do                                               | 2.0                      | 0.18816                                      |
| 3-A-4     | do                               | do                                               | 3.0                      | 0.22912                                      |
| 3-B-1     | Diphenyllauryl monothiophosphate | $C_{12}H_{25}S-P-\left(O-\text{C}_6H_5\right)_2$ | 0.5                      | 0.35328                                      |
| 3-B-2     | do                               | Same as above                                    | 1.0                      | 0.35327                                      |
| 3-B-3     | do                               | do                                               | 2.0                      | 0.21888                                      |
| 3-B-4     | do                               | do                                               | 3.0                      | 0.22528                                      |
| 3-C-1     | Trilauryl trithiophosphate       | $(C_{12}H_{25}S)_3P$                             | 2.0                      | 0.39424                                      |
| 3-C-2     | do                               | $(C_{12}H_{25}S)_2P$                             | 3.0                      | 0.38784                                      |
| Control   |                                  |                                                  | 0                        | 0.44032                                      |

EXAMPLE 4

Twenty-four kinds of quenching oil compositions were prepared by adding phosphates shown in Table 4 below in predetermined amount to 100 weight parts of mineral quenching oil the same as in Example 1.

Roller pins quenched with the above compositions in

70 the same manner as in Example 1 were measured to determine coefficient of boundary friction as in Example 1 with the results shown in Table 5. In Table 5 the mixture described in compositions Nos. 5-C to 5-E are 1:1 weight ratio mixtures of respective compounds.

TABLE 5

| Comp. No.                                  | Name                           | Formula                                                                             | Amount added<br>(wt. parts) | Coefficient of boundary friction<br>(at 50° C.) |
|--------------------------------------------|--------------------------------|-------------------------------------------------------------------------------------|-----------------------------|-------------------------------------------------|
| Zinc dialkyl dithiophosphate added         |                                |                                                                                     |                             |                                                 |
| 5-A-1                                      | Zinc dipentyl dithiophosphate. |    | 0.1                         | 0.33152                                         |
| 5-A-2                                      | do.                            | Same as above                                                                       | 0.3                         | 0.19200                                         |
| 5-A-3                                      | do.                            | do.                                                                                 | 0.5                         | 0.16640                                         |
| 5-A-4                                      | do.                            | do.                                                                                 | 1.0                         | 0.16640                                         |
| 5-A-5                                      | do.                            | do.                                                                                 | 2.0                         | 0.17280                                         |
| 5-A-6                                      | do.                            | do.                                                                                 | 3.0                         | 0.20480                                         |
| 5-B-1                                      | Zinc dihexyl dithiophosphate.  |    | 0.05                        | 0.41600                                         |
| 5-B-2                                      | do.                            | Same as above                                                                       | 0.1                         | 0.23168                                         |
| 5-B-3                                      | do.                            | do.                                                                                 | 0.5                         | 0.15360                                         |
| 5-B-4                                      | do.                            | do.                                                                                 | 1.0                         | 0.14208                                         |
| 5-B-5                                      | do.                            | do.                                                                                 | 2.0                         | 0.16728                                         |
| 5-B-6                                      | do.                            | do.                                                                                 | 3.0                         | 0.17208                                         |
| 5-B-7                                      | do.                            | do.                                                                                 | 4.0                         | 0.18560                                         |
| 5-B-8                                      | do.                            | do.                                                                                 | 5.0                         | 0.18562                                         |
| Mixture—<br>Zinc dibutyl dithiophosphate.  |                                |                                                                                     |                             |                                                 |
| 5-C-1                                      | Zinc dioctyl dithiophosphate.  |    | 0.1                         | 0.41728                                         |
| 5-C-2                                      | Same as Comp. No. 5-C-1.       | Same as Comp. No. 5-C-1.                                                            | 0.3                         | 0.21888                                         |
| 5-C-3                                      | do.                            | do.                                                                                 | 0.5                         | 0.16384                                         |
| 5-C-4                                      | do.                            | do.                                                                                 | 1.0                         | 0.15872                                         |
| 5-C-5                                      | do.                            | do.                                                                                 | 2.0                         | 0.17792                                         |
| 5-C-6                                      | do.                            | do.                                                                                 | 3.0                         | 0.19584                                         |
| Mixture—<br>Zinc dihexyl dithiophosphate.  |                                |                                                                                     |                             |                                                 |
| 5-D-1                                      | Zinc dioctyl dithiophosphate.  |  | 0.1                         | 0.38656                                         |
| 5-D-2                                      | Same as Comp. No. 5-D-1.       | Same as Comp. No. 5-D-1.                                                            | 0.3                         | 0.28672                                         |
| 5-D-3                                      | do.                            | do.                                                                                 | 0.5                         | 0.22400                                         |
| 5-D-4                                      | do.                            | do.                                                                                 | 1.0                         | 0.19200                                         |
| 5-D-5                                      | do.                            | do.                                                                                 | 2.0                         | 0.17280                                         |
| 5-D-6                                      | do.                            | do.                                                                                 | 3.0                         | 0.20992                                         |
| Mixture—<br>Zinc dipropyl dithiophosphate. |                                |                                                                                     |                             |                                                 |
| 5-E-1                                      | Zinc dilauryl dithiophosphate. |  | 0.1                         | 0.38400                                         |
| 5-E-2                                      | Same as Comp. No. 5-E-1.       | Same as Comp. No. 5-E-1.                                                            | 0.3                         | 0.23040                                         |
| 5-E-3                                      | do.                            | do.                                                                                 | 0.5                         | 0.21248                                         |
| 5-E-4                                      | do.                            | do.                                                                                 | 1.0                         | 0.19968                                         |
| 5-E-5                                      | do.                            | do.                                                                                 | 2.0                         | 0.14208                                         |
| 5-E-6                                      | do.                            | do.                                                                                 | 3.0                         | 0.17152                                         |
| Control                                    |                                |                                                                                     | 0                           | 0.44032                                         |

## EXAMPLE 6

Eleven kinds of quenching oil compositions were prepared by adding disulfides shown in Table 6 below in predetermined amount to 100 weight parts of mineral quenching oil the same as in Example 1.

Roller pins quenched with the above compositions in the same manner as in Example 1 were measured to determine coefficient of boundary friction as in Example 1 with the results shown in Table 6.

TABLE 6

| Comp. No. | Name                      | Formula                                                          | Amount added<br>(wt. parts) | Coefficient<br>of boundary<br>friction<br>(at 50° C.) |
|-----------|---------------------------|------------------------------------------------------------------|-----------------------------|-------------------------------------------------------|
| 6-A-1     | Ditertiarybutyl disulfide | $(\text{CH}_3)_3\text{CS}-\text{SC}(\text{CH}_3)_3$              | 0.5                         | 0.2650                                                |
| 6-A-2     | do                        | $(\text{CH}_3)_3\text{CS}-\text{SC}(\text{CH}_3)_3$              | 1.0                         | 0.2957                                                |
| 6-A-3     | do                        | $(\text{CH}_3)_3\text{CS}-\text{SC}(\text{CH}_3)_3$              | 2.0                         | 0.3584                                                |
| 6-B-1     | Dilauryl disulfide        | $\text{C}_{12}\text{H}_{25}\text{S}-\text{SC}_{12}\text{H}_{25}$ | 1.0                         | 0.3520                                                |
| 6-B-2     | do                        | $\text{C}_{12}\text{H}_{25}\text{S}-\text{SC}_{12}\text{H}_{25}$ | 2.0                         | 0.3290                                                |
| 6-C-1     | Diphenyl disulfide        |                                                                  | 0.1                         | 0.33408                                               |
| 6-C-2     | do                        | Same as above                                                    | 0.5                         | 0.38784                                               |
| 6-C-3     | do                        | do                                                               | 1.0                         | 0.40448                                               |
| 6-D-1     | Dibenzyl disulfide        |                                                                  | 0.1                         | 0.33408                                               |
| 6-D-2     | do                        | Same as above                                                    | 0.5                         | 0.38784                                               |
| 6-D-3     | do                        | do                                                               | 1.0                         | 0.40448                                               |
| Control   |                           |                                                                  | 0                           | 0.44032                                               |

## EXAMPLE 7

Seven kinds of quenching oil compositions were prepared by adding tetraalkyl thiuram sulfides shown in Table 7 below in predetermined amount to 100 weight parts of mineral quenching oil the same as in Example 1.

Roller pins quenched with the above compositions in the same manner as in Example 1 were measured to determine coefficient of boundary friction as in Example 1 with the results shown in Table 7 below.

20

## EXAMPLE 8

Twenty-four kinds of quenching oil compositions were prepared by adding carbamates shown in Table 8 below in predetermined amount to 100 weight parts of mineral quenching oil the same as in Example 1.

Roller pins quenched with the above compositions in the same manner as in Example 1 were measured to

TABLE 7

| Comp. No. | Name                            | Formula       | Amount added<br>(wt. parts) | Coefficient<br>of boundary<br>friction<br>(at 50° C.) |
|-----------|---------------------------------|---------------|-----------------------------|-------------------------------------------------------|
| 7-A-1     | Tetramethyl thiuram disulfide   |               | 0.5                         | 0.2790                                                |
| 7-A-2     | do                              | Same as above | 1.0                         | 0.2726                                                |
| 7-A-3     | do                              | do            | 2.0                         | 0.2227                                                |
| 7-B-1     | do                              |               | 0.5                         | 0.2867                                                |
| 7-B-2     | do                              | Same as above | 1.0                         | 0.3046                                                |
| 7-C-1     | Tetramethyl thiuram monosulfide |               | 0.5                         | 0.2010                                                |
| 7-C-2     | do                              | Same as above | 1.0                         | 0.2957                                                |
| Control   |                                 |               | 0                           | 0.44032                                               |

determine coefficient of boundary friction as in Example 1 with the results shown in Table 8 below.

TABLE 8

| Comp. No. | Name                            | Carbamates added | Amount added<br>(wt. parts) | Coefficient<br>of boundary<br>friction<br>(at 50° C.) |
|-----------|---------------------------------|------------------|-----------------------------|-------------------------------------------------------|
| 8-A-1     | Ferric dimethyl dithiocarbamate |                  | 0.5                         | 0.3686                                                |
| 8-B-1     | Cupric dimethyl dithiocarbamate |                  | 0.5                         | 0.2560                                                |
| 8-C-1     | Zinc dimethyl dithiocarbamate   |                  | 0.5                         | 0.2867                                                |
| 8-D-1     | Zinc diethyl dithiocarbamate    |                  | 0.5                         | 0.3136                                                |
| 8-D-2     | do                              | Same as above    | 1.0                         | 0.2778                                                |
| 8-D-3     | do                              | do               | 2.0                         | 0.2453                                                |

TABLE 8—Continued

| Comp. No. | Name                              | Carbamates added                                                                                                                                                              | Amount added (wt. parts) | Coefficient of boundary friction (at 50° C.) |
|-----------|-----------------------------------|-------------------------------------------------------------------------------------------------------------------------------------------------------------------------------|--------------------------|----------------------------------------------|
| 8-E-1     | Zinc dipentyl dithiocarbamate     | $\left[ \begin{array}{c} \text{C}_5\text{H}_{11} & \text{S} \\ & \parallel \\ & \text{N}-\text{C}-\text{S} \\ &   \\ \text{C}_5\text{H}_{11} \end{array} \right]_{\text{Zn}}$ | 0.3                      | 0.40960                                      |
| 8-E-2     | do                                | Same as above                                                                                                                                                                 | 0.5                      | 0.40882                                      |
| 8-E-3     | do                                | do                                                                                                                                                                            | 1.0                      | 0.39296                                      |
| 8-E-4     | do                                | do                                                                                                                                                                            | 2.0                      | 0.39040                                      |
| 8-E-5     | do                                | do                                                                                                                                                                            | 3.0                      | 0.39936                                      |
| 8-F-1     | Cadmium dipentyl dithiocarbamate  | $\left[ \begin{array}{c} \text{C}_5\text{H}_{11} & \text{S} \\ & \parallel \\ & \text{N}-\text{C}-\text{S} \\ &   \\ \text{C}_5\text{H}_{11} \end{array} \right]_{\text{Cd}}$ | 0.25                     | 0.34304                                      |
| 8-F-2     | do                                | Same as above                                                                                                                                                                 | 0.50                     | 0.28544                                      |
| 8-F-3     | do                                | do                                                                                                                                                                            | 1.0                      | 0.28416                                      |
| 8-G-1     | Lead dipentyl dithiocarbamate     | $\left[ \begin{array}{c} \text{C}_5\text{H}_{11} & \text{S} \\ & \parallel \\ & \text{N}-\text{C}-\text{S} \\ &   \\ \text{C}_5\text{H}_{11} \end{array} \right]_{\text{Pb}}$ | 1.0                      | 0.41344                                      |
| 8-G-2     | do                                | Same as above                                                                                                                                                                 | 1.5                      | 0.40704                                      |
| 8-G-3     | do                                | do                                                                                                                                                                            | 2.5                      | 0.37248                                      |
| 8-H-1     | Antimony dipentyl dithiocarbamate | $\left[ \begin{array}{c} \text{C}_5\text{H}_{11} & \text{S} \\ & \parallel \\ & \text{N}-\text{C}-\text{S} \\ &   \\ \text{C}_5\text{H}_{11} \end{array} \right]_{\text{Sb}}$ | 0.25                     | 0.41344                                      |
| 8-H-2     | do                                | Same as above                                                                                                                                                                 | 0.5                      | 0.37504                                      |
| 8-H-3     | do                                | do                                                                                                                                                                            | 1.0                      | 0.32768                                      |
| 8-H-4     | do                                | do                                                                                                                                                                            | 1.5                      | 0.35200                                      |
| 8-H-5     | do                                | do                                                                                                                                                                            | 2.5                      | 0.40192                                      |
| 8-I-1     | Zinc ethylphenyl dithiocarbamate  | $\left[ \begin{array}{c} \text{C}_6\text{H}_5 & \text{S} \\   & \parallel \\ \text{C}_2\text{H}_5 & \text{N}-\text{C}-\text{S} \\   &   \\ & \text{Zn} \end{array} \right]$   | 0.5                      | 0.3418                                       |
| 8-I-2     | do                                | Same as above                                                                                                                                                                 | 1.0                      | 0.3059                                       |
| Control   |                                   |                                                                                                                                                                               | 0                        | 0.44032                                      |

## EXAMPLE 9

Seventeen kinds of quenching oil compositions were prepared by adding mercaptanes shown in Table 9 below in predetermined amount to 100 weight parts of mineral quenching oil the same as in Example 1.

Roller pins quenched with the above compositions in the same manner as in Example 1 were measured to determine coefficient of boundary friction as in Example 1 with the results shown in Table 9 below.

40

## EXAMPLE 10

1.0 weight part of zinc dihexyl dithiophosphate was added to 100 weight parts of three kinds of mineral quenching oils having the following properties to produce the present compositions.

45 Quenching oil used:

- (A) viscosity 66.0 RW sec. at 50° C., flash point 188° C.  
 (B) Viscosity 65.0 RW sec. at 50° C., flash point 186° C.

TABLE 9

| Comp. No. | Name                 | Mercaptanes added                          | Amount added (wt. parts) | Coefficient of boundary friction (at 50° C.) |
|-----------|----------------------|--------------------------------------------|--------------------------|----------------------------------------------|
| 9-A-1     | n-Octyl mercaptane   | $\text{C}_8\text{H}_{17}\text{SH}$         | 0.5                      | 0.3571                                       |
| 9-A-2     | do                   | $\text{C}_8\text{H}_{17}\text{SH}$         | 1.0                      | 0.3341                                       |
| 9-A-3     | do                   | $\text{C}_8\text{H}_{17}\text{SH}$         | 2.0                      | 0.3136                                       |
| 9-B-1     | n-Dodecyl mercaptane | $\text{C}_{12}\text{H}_{25}\text{SH}$      | 0.5                      | 0.3712                                       |
| 9-B-2     | do                   | $\text{C}_{12}\text{H}_{25}\text{SH}$      | 1.0                      | 0.3123                                       |
| 9-B-3     | do                   | $\text{C}_{12}\text{H}_{25}\text{SH}$      | 2.0                      | 0.3048                                       |
| 9-C-1     | n-Cetyl mercaptane   | $\text{C}_{16}\text{H}_{33}\text{SH}$      | 2.0                      | 0.41600                                      |
| 9-C-2     | do                   | $\text{C}_{16}\text{H}_{33}\text{SH}$      | 3.0                      | 0.39296                                      |
| 9-D-1     | Stearyl mercaptane   | $\text{C}_{18}\text{H}_{35}\text{SH}$      | 0.5                      | 0.3814                                       |
| 9-D-2     | do                   | $\text{C}_{18}\text{H}_{35}\text{SH}$      | 1.0                      | 0.3405                                       |
| 9-D-3     | do                   | $\text{C}_{18}\text{H}_{35}\text{SH}$      | 2.0                      | 0.3277                                       |
| 9-E-1     | Thiophenol           | $\text{C}_6\text{H}_5\text{SH}$            | 0.5                      | 0.3098                                       |
| 9-E-2     | do                   | Same as above                              | 1.0                      | 0.2842                                       |
| 9-E-3     | do                   | do                                         | 2.0                      | 0.2406                                       |
| 9-F-1     | Benzyl mercaptane    | $\text{C}_6\text{H}_5\text{CH}_2\text{SH}$ | 0.5                      | 0.3008                                       |
| 9-F-2     | do                   | Same as above                              | 1.0                      | 0.2624                                       |
| 9-F-3     | do                   | do                                         | 2.0                      | 0.2458                                       |
| Control   |                      |                                            | 0                        | 0.44032                                      |

(C) viscosity 775.8 RW sec. at 50° C., flash point 282° C.

Roller pins quenched with the above compositions in the same manner as in Example 1 were measured for coefficient of boundary friction as in Example 1 with the results shown in Table 10 below.

TABLE 10

| Comp. No..   | Quenching oil | Amount of dithiophosphate added | Coefficient of boundary friction at 50° C. |
|--------------|---------------|---------------------------------|--------------------------------------------|
| 10-A.....    | A             | 1.0                             | 0.19480                                    |
| Control..... | A             | 0                               | ( <sup>1</sup> )                           |
| 10-B.....    | B             | 1.0                             | 0.20864                                    |
| Control..... | B             | 0                               | 0.44672                                    |
| 10-C.....    | C             | 1.0                             | 0.17536                                    |
| Control..... | C             | 0                               | ( <sup>1</sup> )                           |

<sup>1</sup> Immeasurable (stopped at third stroke).

## EXAMPLE 11

Bolts made of chromium steel (SAE 5140), 10 mm. in diameter, 27 mm. in length and 1.25 in screw-thread pitch, were heated at 850° C. in nitrogen gas atmosphere and were immediately immersed respectively for 5 minutes in three kinds of the present quenching oil compositions. The resultant cooled bolts were again tempered in a nitrogen gas atmosphere at 500° C. for 2 hours, and respectively immersed in the above quenching oil compositions for 5 minutes.

The fastening force and the fastening torque were measured by a strain gauge with respect to the above resultant bolts to determine the relation therebetween. The results are shown in Table 11, in which the same composition numbers as those in Tables 1 to 9 refer to the same compositions.

TABLE 11

| Torques (kg.-cm.) | Forces (ton) |      |      |      |      |
|-------------------|--------------|------|------|------|------|
|                   | 500          | 600  | 700  | 800  | 900  |
| Comp. No.:        |              |      |      |      |      |
| 2-D-3.....        | 2.15         | 2.70 | 3.25 | 3.75 | 4.40 |
| 5-B-4.....        | 2.33         | 2.90 | 3.43 | 4.13 | 4.80 |
| 6-D-3.....        | 2.35         | 2.80 | 3.10 | 3.54 | 3.98 |
| Control.....      | 1.77         | 2.20 | 2.67 | 2.94 | 3.30 |

As apparent from the foregoing examples, the compositions of the present invention obtained by adding specific compounds included in the groups (I) to (IX) to quenching oils of mineral origin can impart lubricity to quenched metals. None of these compounds will exert any adverse effect on the inherent properties of the quenching oils, provided they are added to the quenching oils in the amount of 0.05 to 5 weight parts based on 100 weight parts of the latter. This is clarified in Table 12 showing the cooling ability of the typical compositions of the present invention as measured in accordance with the method provided in JIS K 2526. The quenching oil used in this test was the same as that in Example 1, the same compositions as those in Tables 1 to 9 being referred to by the same numerals.

TABLE 12

| Comp. No.    | Cooling ability                   |                                                      |
|--------------|-----------------------------------|------------------------------------------------------|
|              | Characteristic temperature (° C.) | Time required for cooling from 800 to 400° C. (sec.) |
| Control..... | 600                               | 2.80                                                 |
| 1-F-2.....   | 600                               | 2.73                                                 |
| 2-F-2.....   | 600                               | 2.83                                                 |
| 3-A-2.....   | 600                               | 2.78                                                 |
| 4-F-1.....   | 600                               | 2.81                                                 |
| 5-B-4.....   | 600                               | 2.54                                                 |
| 6-D-3.....   | 600                               | 2.43                                                 |
| 7-A-2.....   | 600                               | 2.50                                                 |
| 8-F-3.....   | 600                               | 2.78                                                 |
| 9-C-2.....   | 600                               | 2.58                                                 |

What we claim is:

1. A method of simultaneously hardening metal and imparting excellent lubricity to the metal surface which comprises quenching said metal in a quenching oil composition which comprises a mineral quenching oil in major amounts and 0.05 to 5 weight parts, based on 100 weight parts of mineral quenching oil, of at least one zinc dialkyl dithiophosphate having the formula of:



wherein R<sup>7</sup> is an alkyl of 1 to 12 carbon atoms.

2. The method of claim 1 wherein the zinc dialkyl dithiophosphate is at least one species selected from the group consisting of zinc dipropyl dithiophosphate, zinc dibutyl dithiophosphate, zinc dipentyl dithiophosphate, zinc dihexyl dithiophosphate, zinc dioctyl dithiophosphate and zinc dilauryl dithiophosphate.

3. The method of claim 2 in which the zinc dialkyl dithiophosphate is zinc hexyl dithiophosphate.

## References Cited

## UNITED STATES PATENTS

|           |        |                     |               |
|-----------|--------|---------------------|---------------|
| 2,316,080 | 4/1943 | Loane et al. ....   | 252—46.6 X    |
| 2,536,403 | 1/1951 | Wallace et al. .... | 252—32.7 HC X |
| 3,361,668 | 1/1968 | Wiese ....          | 252—32.7 E    |
| 3,657,640 | 3/1971 | Stroh ....          | 252—59        |

## OTHER REFERENCES

Gruse et al.: "Chemical Technology of Petroleum," 3rd ed. (1960), pp. 525-532 and 537.

Handbook of Chemistry and Physics, Rubber Pub. Co., 44th ed. (1962-1963) p. 2252, viscosity conversion graph.

DANIEL E. WYMAN, Primary Examiner

W. H. CANNON, Assistant Examiner

U.S. Cl. X.R.

148—18, 29; 252—32.7 HC, 75